

## UNITED STATES PATENT OFFICE

2,347,572

## ELECTROCLEANING PROCESS

Fred F. Martin, Peoria, and John I. Clark, West Peoria, Ill., assignors to Caterpillar Tractor Co., San Leandro, Calif., a corporation of California

No Drawing. Application March 11, 1940,  
Serial No. 323,392

5 Claims. (Cl. 204—34)

Our invention relates to an electrochemical process for cleaning metallic surfaces, and more particularly to the reclamation or salvaging of a metal employed for application of a protective metallic film on the metal to be cleaned.

A common method employed (in accordance with the teachings of United States patents, Re. 19,773; 1,775,671; 1,867,527; 1,917,022; 1,927,116; 1,954,473; and 1,979,996) for cleaning metal surfaces free of rust or scale, saponifiable and non-saponifiable oils, greases, waxes, and dirt such as paints, carbon smuts or the like, is first to subject the work or metal to be cleaned to a suitable alkaline electrolytic bath, preferably comprising an aqueous solution of tri-sodium phosphate and caustic soda, in which the work is made the anode, and in which are employed substantially insoluble cathodes, such as high silicon iron, known to the trade as "Duriron." Next, the work is subjected to an acid bath, preferably an aqueous solution of sulfuric acid, in which the work is made the cathode and in which are employed both substantially insoluble anode electrodes, such as the previously mentioned high silicon iron, and at least one soluble anode electrode of a metal, such as tin, for applying a protective metal film to the work. Suitable water rinses are generally employed after treatment in each of the electrolytic baths, for washing the work free of electrolytic solution.

The alkaline bath initially serves the purpose of degreasing the work by removal of oily matter and dirt therefrom, while the acid bath performs the function of descaling, the purpose of the deposit of the protective metal film on the work being to shield the work against the acid while the scale is being removed. Frequently, in order to obtain thorough cleansing of the work, it is necessary to subject it to more than one cycle of treatment. In doing this, the work after treatment in the acid bath and with the protective metal film thereon, is subjected to the alkaline bath. Since the work is the anode in such bath, the protective metal will dissolve from the work which thus becomes defilmed; and it accumulates as a heavy spongy deposit on the substantially insoluble cathode electrodes employed in such alkaline bath. Also, under some circumstances when it is desired to omit the protective metal film from the finally treated work, it must be subjected finally to the alkaline bath where, as was previously explained, the protective metal film will dissolve off the work and deposit on the substantially insoluble cathode electrodes. Thus, it is seen that because the alkaline bath serves at first to degrease the work, and then if subjected again to such bath after treatment in the acid bath, to defilm the work free of the film deposited in the acid bath, it serves both as a degreasing and defilming bath.

The acid bath where the protective metal film is deposited on the work must be supplied from time to time with an adequate quantity of the desired metal ions to replenish the supply exhausted by the work. A suitable salt of the desired metal may be added to such bath, but it is more economical to employ the previously mentioned soluble anode of such metal which must be replenished as it is used up. In the case of tin, which is a desirable metal for the purpose because it will alloy with the work while a metal such as lead will not, replacing the soluble anode thereof is quite expensive, by virtue of the relatively high cost of the metal, which according to the latest quotations runs to about 55¢ per pound.

From the preceding, it is seen that in the process as heretofore practiced, there has been a loss, due to the necessity of replenishing the soluble electrode in the acid bath, or supplying a salt of the desired metal in such bath. Our invention is designed to minimize such loss, and has as its objects, among others, the salvaging of the metal employed to deposit a protective film on the work treated in the acid bath, to render more economical a process of the character described. Other objects of our invention will become apparent from a perusal of the following description thereof.

In general, we have found that the substantially insoluble electrodes having the deposit of the protective metal thereon, resulting from treatment of the work in the alkaline degreasing or defilming bath, may be employed as anodes in the acid or descaling bath to replenish the supply of such metal, thus reducing the quantity of soluble anodes of such metal for the acid bath. The material deposits on these electrodes in the degreasing or defilming bath as a spongy sludge which, when tin is employed as the protective metal, will average about 40% tin. Heretofore, it was necessary when the accumulation of sludge became too great, to clean the sludge off; and such sludge was discarded as waste, because it was thought that the metal content thereof was unsatisfactory for replenishing the supply in the acid or descaling bath. Such cleaning was a hard, laborious job requiring considerable time. Thus, it is seen that our process not only salvages the protective metal, but also reduces cost by virtue of elimination of labor heretofore required for cleaning electrodes free of sludge. Instead of employing the electrodes with the protective metal-containing sludge, as anodes in the acid or descaling bath, such protective metal containing sludge may be scraped off and added to the acid bath at suitable intervals to replenish the supply of protective metal, but this is not as desirable as utilizing the electrodes themselves.

In the preferred procedure of our process, tin is utilized as the protective metal, and we re-

place some of the substantially insoluble anode electrodes in the acid or descaling bath by a corresponding number of the substantially insoluble cathode electrodes from the alkaline bath, and which have the tin containing sludge thereon. The anode electrodes taken from the acid bath are similarly substituted for the cathode electrodes taken from the alkaline bath; and in the alkaline bath they will accumulate the tin containing sludge thereon as defilming of the work proceeds. When the acid bath requires further amounts of tin, other electrodes may be similarly interchanged. Thus, the substantially insoluble electrodes are continuously rotated among the baths. The electrodes are usually suspended by hooks on heavy conductor bars, and are consequently readily removable, which enables such interchange or rotation of the substantially insoluble electrodes to be conducted rapidly and with ease.

An electrode having the tin containing sludge thereon taken from the alkaline bath may be used in the acid bath until it is stripped clean of the sludge, and may be then placed back in the alkaline bath. The operator may readily tell, as he has in the past, when the acid bath requires replacement of the supply of tin so that he may rotate the electrodes in the manner described. In this connection, all the tin used in the process can not be salvaged because frequently, the finished work is provided with a protective tin deposit thereon resulting from final treatment in the acid or descaling bath. Therefore, in our process, it is still necessary to supply fresh soluble tin electrodes in the acid bath from time to time.

However, the saving in new protective metal which must be employed is considerable, as can be ascertained from the figures given below showing operations at the plant of our assignee, for the first five months of a year in which the above described salvaging operations were not employed, and the following six months of such year after the salvaging operations were started.

|                                                                           | Jan. 1 to<br>June 1<br>(5 months) | June 1 to<br>Dec. 1<br>(6 months) |
|---------------------------------------------------------------------------|-----------------------------------|-----------------------------------|
| Total weight in pounds of tin bars used as soluble anode in acid solution | 2,080                             | 1,460                             |
| Average weight in pounds of replenishing tin used per month               | 416                               | 243                               |
| Average cost per month at average price of 55¢ per pound                  | \$228.80                          | \$133.65                          |
| Average savings per month                                                 |                                   | \$95.15                           |

With respect to the above data, substantially the same quantity of material was treated in each of the periods compared.

Although we have found our process particularly advantageous in salvaging the tin which is preferably employed, the same salvaging operations may be employed with respect to any other metal, such as lead, which may be applied as a protective film to the work in the acid or descaling bath.

We claim:

1. In the electrochemical process for cleaning metal wherein the metal to be cleaned is the cathode in an electrolytic bath in which a cleaning treatment is effected and which deposits a protective metal film thereon, and the anode in another electrolytic bath in which another cleaning treatment is effected and which removes said protective metal film and deposits the protective metal on a cathode, the step of

salvaging said protective metal which comprises utilizing said cathode with said protective metal deposit thereon as an anode in said first mentioned bath wherein the protective metal deposit is removed and deposited on the metal to be cleaned.

2. In the electrochemical process for cleaning metal wherein the metal to be cleaned is the cathode in a descaling electrolytic bath containing a substantially insoluble anode and a soluble anode of a metal which is deposited as a protective film on said metal to be cleaned, and said metal to be cleaned is the anode in another electrolytic bath which defilms said protective metal film from the metal to be cleaned and deposits the protective metal on a substantially insoluble cathode, the step of salvaging said protective metal which comprises substituting said substantially insoluble cathode with said protective metal deposit thereon for said substantially insoluble anode in said descaling bath whereby said protective metal deposit will be removed in said descaling bath and the metal thereof deposited on said metal to be cleaned.

3. In the electrochemical process for cleaning metal wherein the metal to be cleaned is the cathode in a descaling electrolytic bath containing a plurality of substantially insoluble anode electrodes and a soluble anode of a metal which is deposited as a protective film on said metal to be cleaned, and said metal to be cleaned is the anode in another electrolytic bath which defilms said protective metal film from the metal to be cleaned and deposits the protective metal on a plurality of substantially insoluble cathode electrodes, the step of salvaging said protective metal which comprises rotating said substantially insoluble electrodes by exchanging cathode electrodes with said protective metal deposit thereon for anode electrodes in said descaling bath.

4. In the electrochemical process for cleaning metal wherein the metal to be cleaned is the cathode in an acid electrolytic bath containing a plurality of substantially insoluble anode electrodes and a soluble anode of tin which is deposited as a protective film on said metal to be cleaned, and said metal to be cleaned is the anode in an alkaline electrolytic bath which removes said tin film from said metal to be cleaned and deposits the tin on a plurality of substantially insoluble cathode electrodes, the step of salvaging said tin which comprises replacing substantially insoluble anode electrodes in the acid bath by cathode electrodes in the alkaline bath containing tin deposit thereon.

5. In the electrochemical process for cleaning metal wherein the metal to be cleaned is a cathode in an acid electrolytic bath containing a substantially insoluble anode electrode and a soluble anode of a metal which is deposited as a protective film on the metal to be cleaned, and the metal to be cleaned is an anode in an alkaline electrolytic bath which defilms the protective metal film from the metal to be cleaned and deposits such protective metal on a substantially insoluble cathode electrode, the step of salvaging such protective metal which comprises replacing the substantially insoluble anode electrode in the acid bath by the cathode electrode in the alkaline bath containing the protective metal deposit thereon.